

## 1

2,825,693

## METAL WORKING LUBRICANT

Stewart J. Beaubien, Oakland, Thomas E. Reamer, El Cerrito, and Paul H. Williams, Orinda, Calif., assignors to Shell Development Company, New York, N. Y., a corporation of Delaware

No Drawing. Application February 3, 1955  
Serial No. 486,032

3 Claims. (Cl. 252—32.5)

This invention relates to improved lubricating compositions, and more particularly to aqueous lubricating compositions adapted for various metal cutting and fabricating operations.

The class of water-soluble non-ionic surface active agents available commercially under the trade name "Pluronics," marketed by the Wyandotte Chemical Corporation and of the class of polyoxyalkylene diols described in U. S. Patents 2,674,619 and 2,677,700, have been suggested as suitable lubricants for water-base metal working lubricants. Although cutting fluids containing these surface active agents are excellent as far as cutting and load carrying properties are concerned, it has been found that they cause sticking of machine tool ways, resulting in a slow down, or under aggravated conditions, even in stoppage of production. The reason for this phenomenon is not understood but it appears that it may be attributable to the presence of the hydrophobic homopolymeric polyoxyalkylene unit representing essentially a substantial portion of the molecule. Increasing the water-solubility by incorporating a larger proportion of water-soluble alkylene oxide groups in compounds of this type does not obviate the above undesirable properties which compounds of the above type possess.

The principal object of this invention is to provide an improved aqueous metal-working lubricant. A further object is to provide an aqueous base concentrate suitable as a metal-working lubricant and adapted to be diluted with water to an improved metal working lubricant.

It has now been discovered that the objects of the present invention are attained by a substantially aqueous medium containing a minor amount of (I) a water-soluble heteric copolymeric alkylene glycol, ether or ester thereof, wherein the different oxyalkylene units are substantially randomly distributed throughout the entire polyoxyalkylene chain, and (II) a minor proportion of a water-soluble polyoxyalkylene compound containing a hydrophobic homopolyoxyalkylene unit, of the type described in the above mentioned U. S. Patents 2,674,619 and 2,677,700. These polymeric agents are block copolymers or cogeneric mixtures of conjugated polyoxyalkylene compounds containing at least one hydrophobic homopolyoxyalkylene unit of a unit weight of at least 800, and preferably 900, and one or two other hydrophilic polymeric unit(s) which comprise about 15 to about 90% of the total polymeric compound.

The heteric copolymeric compounds (I) are available commercially under the trade name of "Ucons" and sold by Carbide and Carbon Chemical Company and are fully described in U. S. Patent 2,425,845. The manner in which these compounds (I) function in overcoming the sticking properties of the other type of polymer (II) is not clearly understood. Both polymeric materials (I) and (II) have been suggested in publications and prior patents as additives for metal working compositions. However, polymers of type (I) lack load carrying properties and are therefore relatively useless

## 2

where extreme pressures, wear and loads are encountered and are also excessively corrosive. However, applicants have discovered that the combination of the different types of polymeric compounds (I) and (II) in an aqueous base, provides a lubricant in which the shortcomings of each additive are overcome by the presence of the other; the desirable properties of each are accentuated and the result is an aqueous metal working lubricant which is stable, non-corrosive, does not cause sticking and is capable of carrying loads far in excess of similar compositions but in which either type of additive is omitted.

The heteric copolymeric compounds (I) are water-soluble relatively high molecular weight copolymers containing no substantially hydrophobic polyoxyalkylene units or chains, the polymer being composed of randomly distributed ("heteric") oxyethylene and oxy 1,2-propylene groups in the molecule. Polymers of this type are suitably prepared by the methods described in U. S. Patent 2,425,845, as by reacting aliphatic diols or glycols simultaneously with ethylene oxide and 1,2-propylene oxide. The term "heteric" is used to designate an internal configuration of random distribution of the units making up the copolymer, as distinguished from a grouping of such oxyethylene and oxypropylene units, in homopolymeric units, with those of oxypropylene being of sufficient degree of polymerization to exhibit a substantially hydrophobic character, as in the case of type II polymers.

A suitable method of preparing these heteric copolymers is to charge about 25 to 75% parts of 1,2-propylene glycol and from about 10 to 90 parts ethylene oxide into a suitable reactor and react the mixture in the presence of a caustic catalyst, such as sodium hydroxide. To the mixture a diol such as diethylene glycol is added and the mix is heated to about 110° C. to 120° C. at from 5 to 75 p. s. i. After the reaction is completed, the reaction mixture is neutralized with carbon dioxide and hot water washed. The diol composition phase is dissolved in dichloro diethyl ether and its low-boiling constituents removed by stripping.

## EXAMPLE I

A polymeric product of type (I) is prepared by reacting a mixture of 75 parts of ethylene oxide, 25 parts of 1,2-oxypropylene, 20 parts of diethylene glycol and 1 part of sodium hydroxide. The mixture was heated for 2-4 hours at a temperature of 110°-125° C. and a pressure of 6-40 p. s. i. The product was purified by distillation to remove volatile fraction and filtration to remove sodium hydroxide and had the following properties: average molecular weight 1,108; specific viscosity at 18° C., 0.1811; density, 210° F., 1.0296; refractive index 20° C./D 1.4671; flash temperature, 446° F.; viscosity, centistokes at 210° F., 17.5; and is water-soluble in all proportions.

The second of the polymeric compounds (II) is a block copolymer or cogeneric mixture containing substantially a hydrophobic polyoxyalkylene unit such as polyoxypropylene unit of at least 800 and preferably 900 unit weight and the balance, which comprises from 15 to 90% of the total molecule, being hydrophilic polyoxyalkylene unit or units such as polyoxyethylene units. Copolymers of this type can be prepared by the methods described in U. S. Patents 2,674,619 and 2,677,700. Essentially, these polymeric compounds can be prepared by first condensing an alkylene oxide having from 3 to 8 carbon atoms such as propylene oxide with an organic base compound containing a single or plurality of reactive hydrogen atoms to form a hydrophobic polyoxyalkylene polymer such as polyoxypropylene polymer of at least 800 and preferably 900 molecular weight and thereafter condensing said polymer with ethylene oxide so as to form thereon hydrophilic

polyoxyethylene unit(s) which comprise from about 15% to about 90% of the total polymer.

In preparing the polyoxypropylene polymer, the condensation of propylene oxide with the reactive hydrogen organic compound is normally carried out at elevated temperatures and pressures in the presence of an alkaline catalyst such as sodium alkoxide, a quaternary ammonium base, or sodium hydroxide. Similarly, the condensation reaction may be carried out in the presence of acid catalysts as set forth in U. S. Patent No. 2,510,540.

Although the reaction may be carried out by simply heating a mixture of the reactants under pressure at a sufficiently high temperature this procedure is not ordinarily used as the temperatures and pressures required are excessive and control of the exothermic reaction is difficult.

The preferred method of carrying out the reaction is to add the propylene oxide to a stirred, heated mixture of the desired reactive hydrogen compound and alkaline catalyst in a sealed reaction vessel. By adding the propylene oxide to the reaction vessel at such a rate that it reacts as rapidly as added, an excess of propylene oxide is avoided and control of the reaction is simplified.

The temperature at which the reaction is run will depend upon the particular system in question and especially upon the catalyst concentration used. Generally, at higher catalyst concentrations the reaction can be run at lower temperatures and correspondingly lower pressures. The temperatures and pressures required for any given reaction will vary with the reactive-hydrogen compound, and the type and concentration of catalyst used.

The condensation of ethylene oxide with the polyoxypropylene polymer is carried out in an analogous manner.

The preparation of the type II block polymeric polyoxyalkylene compound is illustrated in Example II.

#### EXAMPLE II.—PART A

In a one-liter 3-neck round bottom flask equipped with a mechanical stirrer, reflux condenser, thermometer and propylene oxide feed inlet, there were placed 57 grams (0.75 mol) of propylene glycol and 7.5 grams of anhydrous sodium hydroxide. The flask was purged with nitrogen to remove air and heated to 120° C. with stirring, and until the sodium hydroxide was dissolved. Then sufficient propylene oxide was introduced into the mixture as fast as it would react until the product possessed a calculated molecular weight of 2380. The product was cooled under nitrogen, the NaOH catalyst neutralized with sulfuric acid and the product filtered to remove inorganic solids. The final product was a water-insoluble polyoxypropylene glycol having an average molecular weight of 1620 as determined by hydroxyl number or acetylation analytical test procedure.

#### EXAMPLE II.—PART B

The foregoing polyoxypropylene glycol, having an average molecular weight of 1620, was placed in the same apparatus as described in Part A of this example, in the amount of 500 grams (0.308 mol), to which there was added 5 grams of anhydrous sodium hydroxide. One hundred and five grams of ethylene oxide was added to an average temperature of 120° C., using the same technique as employed in Part A. The amount of added ethylene oxide corresponded to 17.4% of the total weight of the polyoxypropylene glycol base plus the weight of added ethylene oxide.

Polyoxypropylene is prepared by condensing propylene oxide with a relatively low molecular weight organic compound containing a plurality of reactive hydrogen atoms. The function of this base compound is to furnish reaction hydrogen atoms which initiate the polymerization of the propylene oxide and since the base compound constitutes only a small proportion of the resulting high molecular weight polyoxyalkylene compounds, it ordinarily does not have an influence on the properties thereof. In other words, the particular base compound employed in prepar-

ing the polyoxyalkylene compounds is not critical so long as it furnishes at least one reactive hydrogen atom, and operable polyoxyalkylene compounds are obtained regardless of the particular base compound employed in the preparation of the polyoxypropylene polymer. Ordinarily it is preferred to employ relatively low molecular weight base compounds, e. g., less than 200 molecular weight, preferably polyhydric alcohols, such as ethylene glycol, propylene glycol, butylene glycol, trimethylene glycol, glycerol, and the like, usually a monomeric substance, although dimers, such as diethylene glycol and di-propylene glycol are suitable.

#### EXAMPLE III

- 15 Propylene oxide was condensed separately with acetamide, 1,5-pentanediol, glycerine, ethylene diamine, benzene sulfonamide and sucrose to form polyoxypropylene polymers having molecular weights in excess of 900. The general procedure employed was that of Example II, Part 20 A, except for certain minor changes in technique which will be obvious to those skilled in the art. Ethylene oxide was then condensed with the resulting polyoxypropylene polymers to prepare various compounds suitable for making compositions of the present invention. The compositions of the resulting compounds are set forth in Table I.

Table I

| 30 | Base Compound           | Molecular Weight Polyoxypropylene Polymer (water-insoluble) | Polyoxyethylene Content, Percent of Compound (water-soluble) |
|----|-------------------------|-------------------------------------------------------------|--------------------------------------------------------------|
| 35 | Acetamide.....          | 974                                                         | 36                                                           |
|    | 1,5-pentanediol.....    | 1,372                                                       | 50                                                           |
|    | Glycerine.....          | 2,080                                                       | 48                                                           |
|    | Sucrose.....            | 5,060                                                       | 49                                                           |
|    | Ethylene diamine.....   | 1,850                                                       | 50                                                           |
|    | Benzenesulfonamide..... | 1,179                                                       | 50                                                           |

- 40 In many cases the addition of solubilizing or coupling agents to compositions of this invention is desirable. Suitable agents of this type include: glycol-ethers, such as diethylene glycol monomethyl, ethyl, n- and isopropyl ethers, diethylene glycol mono-butyl ether, diethylene glycol mono-decyl ether, dipropylene glycol monoethyl ether, dipropylene glycol mono-isopropyl ether, dipropylene glycol mono-isoamyl ether, diisobutylene glycol-mono-isopropyl ether, etc. Instead of the glycol-ethers, various alcohols may be used, such as diols having 6 or more carbon atoms in the molecule, e. g., hexylene glycol, decylene glycols, cetylene glycols, etc.; diglycols such as dipropylene glycols, dibutylene glycol, diamylene glycol, ether alcohols and particularly the glycol monalkyl ethers, e. g., 45 Carbon and Carbide Chemical Corp. "Carbitols" and "Cellosolves" such as ethylene glycol mono-ethyl ether, ethylene glycol mono-propyl ether, ethylene glycol mono-n-butyl ether, ethylene glycol mono-isobutyl ether, ethylene glycol mono-tert-butyl ether, ethylene glycol mono-hexyl-butyl ether, propylene glycol mono-isoamyl ether, etc.

50 When necessary, corrosion inhibitors can be used in compositions of this invention of which appreciably water-soluble inorganic or organic nitrites and/or amines such as alkyl or alkyloamines and mixtures thereof are particularly preferred.

55 The nitrites include the metal nitrites such as sodium, potassium, lithium, calcium and barium nitrites, of which the alkali metal nitrites are preferred; also, the organic base nitrites may be used, preferably the organic nitrogen base nitrites, such as benzyl-trimethylammonium nitrite, morpholinium nitrite, dibenzylammonium nitrite, 3,3,5-trimethylcyclohexylammonium nitrite, cyclo-hexylammonium nitrite, beta-phenylethylammonium nitrite, 2,4,5-tetramethyl tetrahydro 1,3-oxazonium nitrite, methyl iso-

butyl carbammonium nitrite, piperidinium nitrite, dicyclohexylammonium nitrite, dicyclohexyl isopropylammonium nitrite, and their homologues and analogues, as well as mixtures containing these and other corrosion inhibitors.

The amines include alkyl and alkylamines such as mono-, di- and triethyl-, propyl-, butylamine; mono-, di- and tri-ethanolamines, dimethyl-ethanolamines, diethyl-ethanolamines, aminoethyl-ethanolamine, mono-, di- and tri-isopropylamine, methyl-diethanolamine, N-acetyl ethanolamine, phenylethanolamine, phenyl-diethanolamine and mixtures thereof.

If desired, oiliness or specific types of anti-wear agents can be added in minor amount to compositions of this invention of which fatty acids and particularly unsaturated fatty acids are most suitable. Among such acids are included saturated acids, e. g., capric, lauric, myristic, palmitic, stearic acids; unsaturated acids such as palmoleic, oleic, ricinoleic, erucic, linoleic, linolenic acids and mixtures thereof. These acids are stably dispersed in the water base apparently by the aid of the block polymers II.

Minor amounts of anti-foaming, masking, bactericidal and anti-corrosive agents for copper and copper alloys, and/or perfuming agents, may be added to improve the composition. Among such materials may be included: anti-foaming agents, e. g., organic silicone compounds illustrated by dimethyl silicone polymer; phosphates, e. g., tributyl phosphate, alkali metal polyphosphates illustrated by sodium alkyl polyphosphates; polyglycidylisopropyl ether (mol. wt. 500-1200, preferably 600-800); masking agents, e. g., low molecular weight aldehydes (acetaldehyde); oil of pines, oil of mirbane; bactericides, e. g., alkyl phenols and phenates such as sodium o-phenyl phenate; and copper anti-corrosion agents, e. g., mercaptobenzothiazoles (sodium mercaptobenzothiazole), and the like.

Effective metal working lubricant concentrates, in accordance with the present invention, are preparable according to the following formulations:

|                                                                                                                                                                                                                                                                     | Broad Range, percent wt. | Preferred Range, percent wt. |
|---------------------------------------------------------------------------------------------------------------------------------------------------------------------------------------------------------------------------------------------------------------------|--------------------------|------------------------------|
| <b>Essential Additives:</b>                                                                                                                                                                                                                                         |                          |                              |
| A block polymer comprising a mixture of a polymeric compound (I) containing a hydrophobic polyoxyalkylene unit of at least 800 mol wt. made by polymeric alkylene oxides from 3 to 8 carbon atoms and polyoxyethylene units comprising 15-99% of the total polymer. | 5-20                     | 6-15                         |
| A randomly distributed water-soluble polyoxypropylene-polyoxyethylene copolymer (I) having substantially no hydrophobic units.                                                                                                                                      | 5-20                     | 6-15                         |
| Preferred Additives:                                                                                                                                                                                                                                                |                          |                              |
| 1. Corrosion inhibitors e. g., inorganic nitrites, alkylamines and mixtures.                                                                                                                                                                                        | 1-12                     | 5-10                         |
| 2. Anti-wear agents, fatty acids, e. g., oleic acid.                                                                                                                                                                                                                | 0.01-5                   | 0.5-3                        |
| Optional Additives:                                                                                                                                                                                                                                                 |                          |                              |
| Anti-foaming agents, coupling agents, germicidal agents, etc.                                                                                                                                                                                                       | 0.01-20                  | 0.1-12                       |
| Base:                                                                                                                                                                                                                                                               | Balance                  | Balance                      |
| Water                                                                                                                                                                                                                                                               |                          |                              |

Illustrative examples of metal working concentrates of this invention comprise:

| Composition A:                              | Percent |
|---------------------------------------------|---------|
| Additive of Example I                       | 10      |
| Additive of Example II                      | 8       |
| Sodium nitrite                              | 8       |
| Triethanolamine                             | 8       |
| Hexylene glycol                             | 10      |
| Oleic acid                                  | 1       |
| Sodium mercaptobenzothiazole (in 50% water) | 0.5     |
| Sodium o-phenylphenate                      | 1       |
| Sodium alkyl polyphosphate                  | 1       |
| Water                                       | Balance |

**Composition B:**

|   |                        |         |
|---|------------------------|---------|
| 5 | Additive of Example I  | 10      |
|   | Additive of Example II | 8       |
|   | Sodium nitrite         | 8       |
|   | Trisodium phosphate    | 8       |
|   | Water                  | Balance |

**Composition C:**

|    |                        |         |
|----|------------------------|---------|
| 10 | Additive of Example I  | 8       |
|    | Additive of Example II | 8       |
|    | Sodium nitrite         | 8       |
|    | Ethanolamine           | 8       |
|    | Water                  | Balance |

**Composition D:**

|    |                        |         |
|----|------------------------|---------|
| 15 | Additive of Example I  | 10      |
|    | Additive of Example II | 10      |
|    | Sodium nitrite         | 8       |
|    | Sodium borate          | 8       |
| 20 | Oleic acid             | 1       |
|    | Dimethylethanolamine   | 8       |
|    | Water                  | Balance |

**Composition E:**

|    |                                             |         |
|----|---------------------------------------------|---------|
| 25 | Additive of Example I                       | 10      |
|    | Additive of Example II                      | 10      |
|    | Sodium nitrite                              | 8       |
|    | Linoleic acid                               | 2       |
| 30 | Triethanolamine                             | 8       |
|    | Sodium mercaptobenzothiazole (in 50% water) | 0.5     |
|    | Water                                       | Balance |

Generally the concentrates can be used neutral or diluted with from 1 to 80 parts of water depending upon the use to which it is put. For cutting of steel, dilutions of 1:20-1:40 are recommended. For cutting of cast iron 1:10-1:20, while for grinding operations dilutions with water of 1:40-1:50, can be used.

Compositions of this invention are outstanding metal

40 working lubricants. For example, composition A (at 1:20 dilution with water) was compared by test to a similar composition but in which additive Example II was omitted (composition X). Composition A showed an increase of 54% in drill life over composition X, and a decrease in sliding friction of from 500 g. to 125 g. over composition X. Also, composition A, when used as a coolant on a lathe in a commercial plant caused no corrosion of metal parts with which it came in contact and the lathe was clean and its working parts were in excellent condition even after weeks of use. However, when a similar composition was used, but in which additive of Example I was omitted (composition Y) in the same machine and operation, the sliding parts of the lathe became sticky and after a day the machine had to be stopped and cleaned.

55 Compositions of this invention can be applied with excellent results to general cutting operations where cooling and lubrication of the tool and work piece under adverse conditions are encountered. Metals machined with the aid of fluids of this invention have good surface finish, are free from rust and stain, and the total life of machine tools and fluid is excellent.

We claim as our invention:

1. A metal working lubricating concentrate comprising 65 a water base composition containing from about 5% to about 20% each of (1) a block copolymer of polyoxypropylene polyoxyethylene compounds containing in their structure hydrophobic oxypropylene groups, hydrophilic oxyethylene groups and an organic radical derived from an organic compound containing a reactive hydrogen atom; the compounds being characterized in that all of the oxypropylene groups are present in polyoxypropylene chains that are attached to the organic radical at the site of a reactive hydrogen atom thereby constituting a hydrophobic polyoxypropylene polymer, the oxyethylene groups

being attached to the polyoxypropylene polymer in polyoxyethylene chains, the average molecular weight of the hydrophobic polyoxypropylene polymers in the mixture being at least 900, as determined by hydroxyl number, and the oxyethylene groups present constituting 15-90% by weight, of total block copolymers, and (2) a mixture of heteric oxyethylene-oxy 1,2-propylene diols in which ethylene oxide and 1,2-propylene oxide are combined therein as oxyethylene and oxy 1,2-propylene groups in a ratio which is at least one-third part of 1,2-propylene oxide for each part of ethylene oxide, by weight, said diols containing in a single molecule both the oxyethylene and the oxy 1,2-propylene groups and said mixture having an average molecular weight of at least 300 attributable to said groups, from about 1% to 12% each of (3) sodium nitrite and an ethanolamine and from about 0.01% to about 5% of (4) an unsaturated high molecular weight fatty acid.

2. A metal working lubricating concentrate comprising a water base composition containing from about 5% to about 20% each of (1) a block copolymer of polyoxypropylene-polyoxyethylene containing in their structure oxypropylene groups, oxyethylene groups and an organic radical derived from an organic compound containing a plurality of reactive hydrogen atoms; the compounds being characterized in that all of the oxypropylene groups are present in polyoxypropylene chains that are attached to the organic radical at the site of a reactive hydrogen atom thereby constituting a hydrophobic polyoxypropylene polymer; the oxyethylene groups being attached to the polyoxypropylene polymer in hydrophilic polyoxyethylene chains; the average molecular weight of the hydrophobic polyoxypropylene polymers in the mixture being at least 1600, as determined by hydroxyl number, and the oxyethylene groups present constituting 30-60% by weight, of the mixture, and (2) a mixture of heteric oxyethylene-oxy 1,2-propylene diols in which ethylene oxide and 1,2-propylene oxide are combined therein as oxyethylene and oxy 1,2-propylene groups in a ratio which is at least one-third part of 1,2-propylene oxide for each part of ethylene oxide, by weight; said diols containing in a single molecule both the oxyethylene and the oxy 1,2-propylene groups and said mixture having an average molecular weight of at least 300 attributable to said groups; from about 1% to 12% each of 45

(3) sodium nitrite, (4) triethanolamine, (5) hexylene glycol, and from about 0.01% to about 5% each of (6) oleic acid, (7) sodium o-phenylphenate, (8) sodium alkyl polyphosphate and (9) sodium mercaptobenzothiazole.

3. A metal working lubricating concentrate consisting essentially of a water base composition containing: (1) 10% of a block copolymer of polyoxypropylene-polyoxyethylene containing in its structure oxypropylene groups, oxyethylene groups and an organic radical derived from an organic compound containing a plurality of reactive hydrogen atoms, the copolymer being characterized in that all of the oxypropylene groups are present in polyoxypropylene chains that are attached to the organic radical at the site of a reactive hydrogen atom thereby constituting a hydrophobic polyoxypropylene polymer structure, the oxyethylene groups being attached to the polyoxypropylene polymer structure in hydrophilic polyoxyethylene chains, the average molecular weight of the hydrophobic polyoxypropylene polymer structure in the copolymer being at least 1600, as determined by hydroxyl number, and the oxyethylene groups present constituting 30-60% by weight of the copolymer, (2) 8% of a mixture of heteric oxyethylene-oxy-1,2-propylene diols in which oxyethylene and oxy-1,2-propylene groups are present in a ratio which is at least one-third part by weight of oxy-1,2-propylene groups for each part by weight of oxyethylene groups, said diols containing in a single molecule both the oxyethylene and the oxy-1,2-propylene groups and having an average molecular weight of at least 300 attributable to said groups, (3) 8% sodium nitrite, (4) 8% triethanolamine, (5) 10% hexylene glycol, (6) 1% oleic acid, (7) 1% sodium o-phenylphenate, (8) 1% sodium alkyl polyphosphate and (9) 1/2% sodium mercaptobenzothiazole.

#### References Cited in the file of this patent

#### UNITED STATES PATENTS

|           |           |       |               |
|-----------|-----------|-------|---------------|
| 2,425,845 | Toussaint | ----- | Aug. 19, 1947 |
| 2,692,859 | Talley    | ----- | Oct. 26, 1954 |

#### FOREIGN PATENTS

|         |               |       |              |
|---------|---------------|-------|--------------|
| 716,354 | Great Britain | ----- | Oct. 6, 1954 |
| 721,526 | Great Britain | ----- | Jan. 5, 1955 |